

## UNITED STATES PATENT OFFICE

2,249,698

## ROOFING AND THE LIKE

Richard A. Wilkins, Rome, N. Y., assignor to Revere Copper and Brass Incorporated, Rome, N. Y., a corporation of Maryland

No Drawing. Application March 28, 1941,  
Serial No. 385,681

3 Claims. (Cl. 108—13)

My invention relates to roofing and the like, and particularly to improvements in the roofing forming the subject matter of my pending applications Serial Number 363,515, filed October 30, 1940, and Serial Numbers 381,697 and 381,698, both filed March 4, 1941.

As pointed out in the above mentioned pending applications, the material heretofore commonly employed for copper roofing, sheathing, and other exposed protective coverings for buildings has been thin rolled sheets of highly refined copper. Further, in refining copper for these purposes it has heretofore always been the practice of producers thereof to remove so far as possible all impurities so as to secure as pure a copper as possible. The known high resistance of pure copper generally to chemical corrosion, and the observed fact that impurities commonly found in rolled copper tend to make it less ductile in both the hot and cold rolled conditions, more difficult to produce by either hot or cold rolling, and commonly "cold short" in the sense that it tends to crack when bent or otherwise cold worked, have caused pure copper heretofore to be considered the most satisfactory commercially available material for light weight metal roofing and the like. In fact during the past forty years copper roofing has for these reasons been made almost exclusive of electrolytically refined copper, which commonly is 99.9% pure copper.

Nevertheless it is a frequently observed fact that copper roofing, even when substantially 100% pure electrolytically refined copper, often fails in use, being subject to cracking sufficient to render it non-waterproof. Heretofore it was believed that these cracks were caused by mechanical fatigue resulting by reason of the cyclic stresses set up by alternate expansion and contraction of the copper sheets under varying temperature conditions. For that reason builders heretofore have resorted to expensive roof constructions, and various expensive expedients such as corrugating the roofing and the employment of elaborately designed expansion joints, and the use of heavy gauge copper in the attempt to relieve or reduce the effect on the roofing of these cyclic stresses and thereby eliminate so far as possible this form of failure. Although these attempts have been partially successful, the expense incidental thereto, and the many failures which actually have occurred in spite of these precautions, have seriously interfered with the general adoption of this otherwise very satisfactory roofing.

As pointed out in applicant's pending applica-

tions above referred to, applicant has found that the failure of copper roofing and the like heretofore has not been correctly understood. This material, he has found, does not fail primarily by reason of the cyclic stresses to which it is subjected when in use, as heretofore believed, but, strangely enough, primarily by reason of a heretofore wholly unsuspected type of corrosion which occurs when this highly pure copper is exposed to an atmosphere contaminated by wind borne products of combustion of modern domestic and industrial fuel burning appliances and industrial atmospheres in general.

Applicant has found, that upon removing the patina and other accumulated corrosion products from copper roofing which has failed, the copper roofing surface thus exposed is characteristically pitted, instead of being in its smooth unpitted condition in which it originally left the rolling mill or the metal showing a uniform decrease in thickness over its whole surface due to corrosion.

His investigations show that these pits are caused by the formation on the copper, when exposed to a contaminated atmosphere, of a film of corrosion products which is characterized by a lack of adhesion to the copper, a lack of tenacity in respect to failure, and a tendency toward perviousness which allow the copper to be attacked locally rather than uniformly by the corrosive media and thereby result in the formation of sharply defined, inwardly pointed pits in the nature of notches. He has found that copper so attacked rapidly fails when subjected to the cyclic stresses hereinbefore referred to by reason of the natural tendency of the stresses to be concentrated in the metal below the bottoms of the notch-like pits. As a result of this concentration of the stresses, the metal below the bottoms of the pits "work hardens" and the fatigue strength of the material is exceeded, and as a result the metal cracks at the pits.

Pure copper roofing applicant has found is comparatively sensitive to this "notch effect," when caused by a combination of chemical corrosion and subjection to cyclic stresses, on account of the film which forms on it causing the pure copper to pit and the great sensitivity of pure copper to work hardening when cold worked.

The above mentioned applications point out that this type of failure of copper roofing as constructed from thin sheets, commonly from 0.003 to 0.03 inch in thickness, can be substantially entirely avoided by incorporating into the copper controlled amounts of arsenic or antimony, or both.

When either arsenic or antimony, or both, are incorporated in proper amounts it has been found that the surface of the copper, after the patina or other accumulated products of corrosion are removed, is in an unpitted condition, any corrosion which has occurred being substantially uniformly distributed over its surface. Also it has been found that either arsenic or antimony, or both, most markedly decrease the sensitivity of the copper to work hardening when cold worked, and therefore any scratches, dents, or the like in the nature of notches which might be formed during the handling or installation of the roofing will not cause it to fail by reason of notch defect. In other words, the action of these substances on the roofing is twofold: it prevents notches from being formed by corrosion and prevents the roofing failing by notch effect even if the notches are accidentally formed by mechanical means.

It has been found that the presence of the proper amounts of arsenic or antimony, or both, in the copper roofing produces on the roofing surface a corrosion film which is tenacious, adherent, impervious and non-hygrosopic, the film being comparably as ductile as the copper base material itself, thus permitting the roofing to be repeatedly bent without rupture of the film or interruption of its adherence to the copper. Thus this film effectively protects the underlying base material from contaminated air and moisture, and in this way effectively eliminates the possibility of the formation of the above mentioned notch-like pits, for any slight amount of corrosion which occurs will be uniformly distributed over the surface of the copper. Most importantly this film has the property of being self-healing in the sense that if for any reason its continuity is locally interrupted it will rapidly reform when subjected to corrosion and thus act to prevent substantial local corrosion at the interrupted regions which in a pure copper would continue to corrode at an accelerated rate resulting in pitting at the point of interruption of the film.

Applicant has now found that phosphorus may be substituted for arsenic or antimony, or a combination of the two, to produce in general the same effects, namely, to produce on the copper roofing surface, when subjected to atmospheric corrosion, an instantly self-healing, tenacious, adherent, impervious, non-hygrosopic film, apparently formed of a phosphorus content compound, while rendering the copper roofing less sensitive to failure by reason of notch effect than sheet copper without the phosphorus when subjected to the cyclic stresses caused by expansion and contraction of the roofing. The film which forms when phosphorus is present, however, is thicker, and self-heals more quickly, than the films caused by the presence of arsenic or antimony, or both. Further, phosphorus, it has been found, has the most important effect of very markedly reducing the heat conductivity of the copper roofing, this reduction in heat conductivity being as low as 50% of that of pure copper in some instances within the range that will produce the other desirable effects. Because phosphorus produces this improved film and increases the insulating effect of the roofing, and further because the film is of a pleasing brownish black appearance, makes the roofing solder more easily, and increases the tensile and fatigue strengths of the copper roofing and in general its ductility,

its use, it has been found, is very desirable in this connection.

It has been found that within the ranges of 0.1 to 1% phosphorus the copper has a greater tensile strength and is more ductile when cold than pure copper, the tensile strength increasing with the amount of phosphorus. Phosphorus within this range also increases the fatigue strength of the copper roofing, the fatigue strength being at a maximum at about 0.4 to 0.5% phosphorus. The resistance to work hardening and to failure by reason of notch effect is also increased by additions of phosphorus within the range of 0.1 to 1%, being at a maximum at about 0.4 to 0.6%. Throughout the range of 0.1 to 1% phosphorus the tenacious, self-healing, adherent, protective film forms, and the copper can be commercially hot and cold worked into roofing sheets.

When adding phosphorus best results ordinarily will be secured if the roofing does not contain impurities which tend to render it less malleable in the hot and cold conditions and thus tend to cause the hot or cold rolling or other working of the roofing during its fabrication to result in sub-microscopic surface cracks therein analogous in their effects to pits.

Among these deleterious substances are lead, bismuth, iron, nickel and sulphur, very small amounts of all of which tend to make the copper roofing more difficult to produce, and all of which tend to make the copper roofing containing phosphorus approach the poor resistance of pure copper roofing to corrosion and its sensitivity to notch effect, and thereby act to destroy the beneficial effects of the phosphorus. The presence of such substances as cobalt, tin, silicon and zinc in substantial amounts had also best be avoided as they tend to increase the sensitivity of the copper roofing to work hardening and notch effect. Thus it will be understood, that in the sense the copper roofing does not contain deleterious substances or amounts thereof which substantially destroy the beneficial effects tended to be imparted by the phosphorus, the balance 45 of the alloy aside from the phosphorus is essentially copper.

In making the roofing according to the invention the copper may be melted, and the phosphorus added to the melt in the form of phosphor-copper. The molten metal may then be cast into slabs, which latter may be rolled into sheets of desired thickness by the usual mill process of rolling copper roofing sheets. Finally the rolled sheets may be annealed to the degree 55 of softness that will best resist the cyclic stresses to which they are subjected when in use.

For convenience in terminology the article of manufacture according to the invention is termed "roofing," it being understood that as used in the appended claims such term includes various shingles, sheathings, valleys, and like protective coverings for buildings, as well as what in a more limited sense is ordinarily termed "roofing." Also it will be understood that the roofing according to the invention comprises sheet copper presenting an extensive external roofing surface, and may in this sense consist of a backing having an exterior sheet of copper as well as consist wholly of sheet copper.

70 I claim:

1. Roofing comprising sheet copper presenting an extensive external roofing surface, the copper being alloyed with such amount of phosphorus between 0.1 and 1% as will cause the formation on said surface when exposed to atmospheric

corrosion of a self-healing, adherent, protective film composed predominantly of phosphorus content compound, while rendering the sheet copper less sensitive to failure by reason of notch effect than sheet copper without the phosphorus when subjected to the cyclic stresses caused by expansion and contraction of the roofing.

2. Roofing comprising sheet copper presenting an extensive external roofing surface, the copper

being alloyed with approximately 0.1 to 1% phosphorus, the balance of the alloy in respect to the phosphorus being essentially copper.

3. Roofing comprising sheet copper presenting an extensive external roofing surface, the copper being alloyed with approximately 0.4 to 0.6% phosphorus, the balance of the alloy in respect to the phosphorus being essentially copper.

RICHARD A. WILKINS.

CERTIFICATE OF CORRECTION.

Patent No. 2,249,698.

July 15, 1941.

RICHARD A. WILKINS.

It is hereby certified that error appears in the printed specification of the above numbered patent requiring correction as follows: Page 2, first column, line 15, for the word "defect" read --effect--; and that the said Letters Patent should be read with this correction therein that the same may conform to the record of the case in the Patent Office.

Signed and sealed this 16th day of September, A. D. 1941.

(Seal)

Henry Van Arsdale,  
Acting Commissioner of Patents.